



US011817288B2

(12) **United States Patent**  
**Allaedini**

(10) **Patent No.:** US 11,817,288 B2  
(45) **Date of Patent:** Nov. 14, 2023

(54) **GRAPHITE X-RAY WINDOW**

(71) Applicant: **Moxtek, Inc.**, Orem, UT (US)

(72) Inventor: **Ghazaleh Allaedini**, Orem, UT (US)

(73) Assignee: **Moxtek, Inc.**, Orem, UT (US)

(\*) Notice: Subject to any disclaimer, the term of this patent is extended or adjusted under 35 U.S.C. 154(b) by 0 days.

(21) Appl. No.: **17/887,713**

(22) Filed: **Aug. 15, 2022**

(65) **Prior Publication Data**

US 2023/0082103 A1 Mar. 16, 2023

**Related U.S. Application Data**

(60) Provisional application No. 63/243,846, filed on Sep. 14, 2021.

(51) **Int. Cl.**

**H01J 35/18** (2006.01)

**H01J 5/18** (2006.01)

(52) **U.S. Cl.**

CPC ..... **H01J 35/18** (2013.01); **H01J 5/18** (2013.01); **H01J 2235/183** (2013.01)

(58) **Field of Classification Search**

CPC ..... H01J 5/18; H01J 35/18; H01J 2235/183  
See application file for complete search history.

(56) **References Cited**

**U.S. PATENT DOCUMENTS**

2013/0051535 A1 \* 2/2013 Davis ..... H01J 5/18  
264/400  
2013/0094629 A1 \* 4/2013 Liddiard ..... H01J 35/18  
378/140

\* cited by examiner

*Primary Examiner* — Anne M Hines

(74) *Attorney, Agent, or Firm* — Thorpe North & Western, LLP.

(57) **ABSTRACT**

The x-ray windows herein can have low gas permeability, low outgassing, high strength, low visible and infrared light transmission, high x-ray flux, low atomic number materials, corrosion resistance, high reliability, and low-cost. The x-ray window can include a film 11 with a polymer layer 22 and a graphite layer 21. The film 11 can consist essentially of graphite and polymer. Most of the film 11 can be the graphite layer 21. The polymer layer 22 can be a small portion of the film 11.

**20 Claims, 4 Drawing Sheets**





*Fig. 1*



*Fig. 2*



*Fig. 3*





*Fig. 6*



*Fig. 7*



*Fig. 8*



*Fig. 9*



*Fig. 10*

## 1

## GRAPHITE X-RAY WINDOW

## CLAIM OF PRIORITY

This application claims priority to U.S. Provisional Patent Application No. 63/243,846, filed on Sep. 14, 2021, which is incorporated herein by reference.

## FIELD OF THE INVENTION

The present application is related to x-ray windows.

## BACKGROUND

X-ray windows are designed to transmit a high percent of x-rays, including low energy x-rays. X-ray windows are used in expensive systems requiring high reliability. High system requirements result in demanding characteristics of the x-ray window.

## BRIEF DESCRIPTION OF THE DRAWINGS

(Drawings Might not be Drawn to Scale)

FIG. 1 is a cross-sectional side-view of an x-ray window 10 with a film 11. The film 11 can be made mostly of carbon, such as graphite.

FIG. 2 is a cross-sectional side-view of an x-ray window 10 with a film 11. The film can include a polymer layer 22 and a graphite layer 21.

FIG. 3 is a cross-sectional side-view of an x-ray device 30 comprising an x-ray window 10 mounted to a frame 31. The x-ray window 10 can include a film 11 spanning an aperture 32 of the frame 31.

FIG. 4 is a cross-sectional side-view of an x-ray device 40 comprising an x-ray window 10 mounted on a housing 41. The x-ray window 10 can include a film 11 spanning an aperture 42 of the housing 41. The film 11 can include a polymer layer 22 facing a vacuum at an interior 44 of the housing 41, and a graphite layer 21 facing ambient pressure at an exterior 43 of the housing 41.

FIG. 5 is a perspective-view of a step 50 in a method of making an x-ray window, including obtaining a graphite layer 21 on a flexible substrate 51.

FIG. 6 is a perspective-view of a step 60 in a method of making an x-ray window, including spin coating a polymer precursor 63 on the graphite layer 21.

FIG. 7 is a perspective-view of a step 70 in a method of making an x-ray window, including baking the flexible substrate 51, the graphite layer 21, and the polymer precursor 63 to form a polymer layer 22 (see FIG. 6) on the graphite layer 21.

FIGS. 8-9 are perspective-views of steps 80-90 in a method of making an x-ray window, including laser cutting the polymer layer 22, the graphite layer 21, and the flexible substrate 51 to form multiple x-ray windows.

FIG. 10 is a perspective-view of a step 100 in a method of making an x-ray window, including removing the flexible substrate 51 from the graphite layer 21.

## DEFINITIONS

The following definitions, including plurals of the same, apply throughout this patent application.

As used herein, the terms "on", "located on", "located at", and "located over" mean located directly on or located over with some other solid material between. The terms "located

## 2

directly on", "adjoin", "adjoins", and "adjoining" mean direct and immediate contact.

As used herein, the term "nm" means nanometer(s) and the term "μm" means micrometer(s).

## Detailed Description

Useful characteristics of x-ray windows include low gas permeability, low outgassing, high strength, low visible and infrared light transmission, high x-ray flux, low atomic number materials, corrosion resistance, high reliability, and low-cost. Each x-ray window design is a balance between these characteristics.

An x-ray window can combine with a housing to enclose an internal vacuum. The internal vacuum can aid device performance. For example, an internal vacuum for an x-ray detector (a) minimizes gas attenuation of incoming x-rays and (b) allows easier cooling of the x-ray detector.

Permeation of a gas through the x-ray window can degrade the internal vacuum. Thus, low gas permeability is a desirable x-ray window characteristic.

Outgassing from x-ray window materials can degrade the internal vacuum of the device. Thus, selection of materials with low outgassing is useful.

The x-ray window can face vacuum on one side and atmospheric pressure on an opposite side. Therefore, the x-ray window may need strength to withstand this differential pressure.

Visible and infrared light can cause undesirable noise in the x-ray detector. The ability to block transmission of visible and infrared light is another useful characteristic of x-ray windows.

High x-ray flux through the x-ray window allows (a) rapid functioning of the x-ray detector and (b) increased x-ray flux out of an x-ray tube. Therefore, high x-ray transmissivity through the x-ray window is useful.

Detection and analysis of low-energy x-rays is needed in some applications. High transmission of low-energy x-rays is thus another useful characteristic of x-ray windows.

X-rays can be used to analyze a sample. X-ray noise from surrounding devices, including from the x-ray window, can interfere with a signal from the sample. X-ray noise from high atomic number materials are more problematic. It is helpful, therefore, for the x-ray window to be made of low atomic number materials.

X-ray windows are used in corrosive environments, and may be exposed to corrosive chemicals during manufacturing. Thus, corrosion resistance is another useful characteristic of an x-ray window.

X-ray window failure is intolerable in many applications. For example, x-ray windows are used in analysis equipment on Mars. High reliability is a useful x-ray window characteristic.

X-ray window customers demand low-cost x-ray windows with the above characteristics. Reducing x-ray window cost is another consideration.

The x-ray windows 10 described herein, and x-ray windows manufactured by the methods described herein, can have these useful characteristics (low gas permeability, low outgassing, high strength, low visible and infrared light transmission, high x-ray flux, low atomic number materials, corrosion resistance, high reliability, and low-cost). Each example may satisfy one, some, or all of these useful characteristics.

As illustrated in FIGS. 1-4, an x-ray window 10 is shown including a film 11. The film can be planar across its entire width. The film 11 can include graphite and polymer. The

film 11 can include other materials. Preferably, the film 11 is solely graphite, mostly graphite, or graphite plus a thin layer of polymer. The film 11 can be made mostly or solely of carbon. The film 11 can consist of carbon, hydrogen, nitrogen, and oxygen.

The film 11 can have  $\geq 70$ ,  $\geq 80$ ,  $\geq 85$ ,  $\geq 90$ ,  $\geq 95$ ,  $\geq 99$  mass percent carbon. The film 11 can have  $\leq 99$ ,  $\leq 99.5$ , or  $\leq 99.9$  mass percent carbon. The mass percent carbon value ranges of this paragraph can be such value ranges across the entire film 11 or across an aperture 32 or 42 of a frame 31 or housing 41 (see FIGS. 3 and 4).

The film 11 can be thin to improve x-ray transmission. For example, the film 11 can have a maximum thickness T11 that is in one of the following ranges:  $T11 \leq 15 \mu\text{m}$ ,  $T11 \leq 25 \mu\text{m}$ ,  $T11 \leq 50 \mu\text{m}$ ,  $T11 \leq 100 \mu\text{m}$ , or  $T11 \leq 400 \mu\text{m}$ .

The film 11 can be thick to provide sufficient strength to span an aperture 32 or 42 (see FIGS. 3 & 4). For example, the film 11 can have a maximum thickness T11 that is in one of the following ranges:  $1 \mu\text{m} \leq T11$ ,  $3 \mu\text{m} \leq T11$ ,  $5 \mu\text{m} \leq T11$ , or  $8 \mu\text{m} \leq T11$ .

The maximum thickness T11 value ranges of the prior two paragraphs can be such value ranges across the entire film 11 or just across a portion spanning an aperture 32 (see FIG. 3).

As illustrated in FIG. 2, the film 11 can include a polymer layer 22 on a graphite layer 21. The polymer layer 22 can adjoin the graphite layer 21. The film 11 can consist essentially of graphite and polymer.

The graphite layer 21 can include  $\geq 80$ ,  $\geq 85$ ,  $\geq 90$ ,  $\geq 95$ ,  $\geq 99$ , or  $\geq 99.9$  mass percent carbon. The polymer layer 22 can include polyimide.

The polymer layer 22 can be thinner than the graphite layer 21. For example,  $T21/T22 > 1$ ,  $T21/T22 \geq 10$ ,  $T21/T22 \geq 50$ , or  $T21/T22 \geq 75$ , where T21 is a thickness of the graphite layer 21 and T22 is a thickness of the polymer layer 22. As another example,  $T21/T22 \leq 150$ ,  $T21/T22 \leq 200$ ,  $T21/T22 \leq 500$ , or  $T21/T22 \leq 1000$ . Example thicknesses of the graphite layer 21 include  $1 \mu\text{m} \leq T21$ ,  $2 \mu\text{m} \leq T21$ ,  $5 \mu\text{m} \leq T21$ , or  $10 \mu\text{m} \leq T21$ ; and  $T21 \leq 14 \mu\text{m}$ ,  $T21 \leq 20 \mu\text{m}$ ,  $T21 \leq 40 \mu\text{m}$ ,  $T21 \leq 60 \mu\text{m}$ , or  $T21 \leq 100 \mu\text{m}$ . Example thicknesses of the polymer layer 22 include  $10 \text{ nm} \leq T22$ ,  $20 \text{ nm} \leq T22$ ,  $50 \text{ nm} \leq T22$ , or  $80 \text{ nm} \leq T22$ ; and  $T22 \leq 120 \text{ nm}$ ,  $T22 \leq 250 \text{ nm}$ ,  $T22 \leq 500 \text{ nm}$ , or  $T22 \leq 2 \mu\text{m}$ .

Combining a thick graphite layer 21 with a very thin polymer layer 22 is preferred for achieving the characteristics desirable described above. These characteristics are preferably achieved by a film 11 that consists essentially of the graphite layer 21 and the polymer layer 22. These characteristics are preferably achieved through the method described below.

As illustrated in FIG. 3, x-ray device 30 can comprise an x-ray window 10 mounted to a frame 31. The x-ray window 10 can include a film 11, as described above. The film 11 can span an aperture 32 of the frame 31. The aperture 32 can be void of solid material except for the film 11. The film 11 can be the only solid structure spanning the aperture 32 of the frame 31.

As illustrated in FIG. 4, x-ray device 40 can comprise an x-ray window 10 mounted to a housing 41. The x-ray window 10 can include a film 11, as described above. The film 11 can span an aperture 42 of the housing 41. The aperture 42 can consist essentially of the film 11. The film 11 can be the only solid structure spanning the aperture 42 of the housing 41.

An interior 44 of the housing 41 can be a vacuum. An exterior 43 of the housing 41 can be ambient pressure. The film 11 can include a polymer layer 22 facing the vacuum at the interior 44, and a graphite layer 21 facing the ambient

pressure at the exterior 43. This arrangement is preferred for reducing outgassing of material of the x-ray window 10 into the vacuum of the interior 44 of the housing 41.

Following are example characteristics of the film 11:

5  $T21/T22 = 120$ ,  $T21 = 12 \mu\text{m}$ ,  $T22 = 100 \text{ nm}$ ,  $T11 = 12.1 \mu\text{m}$ . The film 11 can have about 99.7% mass percent carbon. The polymer layer 22 can be polyimide. The film 11 can consist essentially of the graphite layer 21 and the polymer layer 22 across the aperture 42.

10 Method

A Method of Making an x-Ray Window can Include Some or all of the Following Steps:

15 Step 50 (FIG. 5) includes obtaining a graphite layer 21 on a flexible substrate 51. The flexible substrate 51 can include vinyl or polyethylene terephthalate. A thickness T51 of the flexible substrate 51 divided by a thickness T21 of the graphite layer 21 can be at least 2 and not greater than 20 ( $2 \leq T51/T21 \leq 20$ ). One example of a graphite layer 21 on a 20 flexible substrate 51 is DSN5012 by DASEN/thermalgraphite.com.

25 Step 60 (FIG. 6) includes spin coating a polymer precursor 63 on the graphite layer 21. A dispenser 62 of the polymer precursor 63 is shown in FIG. 6. This can be a pipette or syringe for manual application, or it can be a dropper of an automated tool. The flexible substrate 51 can face a spin coat tool 61 and the graphite layer 21 can face away from the spin coat tool 61. A spin plate on the spin coat tool 61 can comprise silicon. The flexible substrate 51 can 30 adjoin the silicon spin plate.

35 The polymer precursor 63 can include an imide dissolved in N-methyl-2-pyrrolidone. The imide can be biphenyldianhydride/1,4 phenylenediamine. A volume of the N-methyl pyrrolidone divided by a volume of the imide can be  $\geq 1.5$  and  $\leq 6$ . Baking step 70 can form the imide into a polyimide in the polymer layer 22.

40 Step 70 (FIGS. 7-8) includes baking the graphite layer 21 and the polymer precursor 63 to form a polymer layer 22 on the graphite layer 21. A hot plate 71 is shown in FIG. 7. After this baking step. The flexible substrate 51 can face the hot plate 71. Alternatively, an oven may be used.

45 The polymer precursor 63 is shown in FIG. 7, which is formed into the polymer layer 22 by the bake, as shown in FIG. 8. In step 70, baking can also include baking the flexible substrate 51.

50 Steps 80-90 (FIGS. 8-9) include laser cutting the polymer layer 22 and the graphite layer 21 to form multiple x-ray windows. In steps 80-90, the polymer layer 22 and the graphite layer 21 can be cut together in a single step by the laser 82. The flexible substrate 51 can also be cut together with the polymer layer 22 and the graphite layer 21 by the laser 82. An Nd:YAG laser may be used to cut the polymer layer 22, the graphite layer 21, and the flexible substrate 51.

55 Step 100 (FIG. 10) includes removing the flexible substrate 51 from the graphite layer 21. In step 100, the flexible substrate 51 can be removed from the graphite layer 21 by manually peeling it off. Plastic-tip tweezers are preferred. The flexible substrate 51 can be removed (step 100) from the graphite layer 21 after baking (step 70), after cutting (steps 60 80-90), or after both. Performing steps 70, 80, 90, and 100 in this order can reduce the chance of damage to the film 11.

65 The steps of the method can be performed in the above order, or other order if so specified in the claims. Some of the steps can be performed simultaneously unless explicitly noted otherwise in the claims. Components of the x-ray window, made by this method, can have properties as described above the method description.

## 5

Here are steps of one example method: DSN5012 is used for the graphite layer **21** and the flexible substrate **51**. The flexible substrate **51** is a 75  $\mu\text{m}$  thick layer of polyethylene terephthalate. The graphite layer **21** is 12  $\mu\text{m}$  thick. The polymer precursor **63** is biphenyldianhydride/1,4-phenylenediamine dissolved in N-methyl-2-pyrrolidone, in a 1:3 ratio. A spin coat tool **61** with a silicon wafer is used, with the flexible substrate **51** adjoining the silicon wafer. The film **11** is baked on a hot plate about 80° C. for 10 minutes, then left to cure for 24 hours at room temperature. The film **11** is then laser cut by an Nd:YAG laser. Tweezers are then used to peel the flexible substrate **51** off of the graphite layer **21**.

What is claimed is:

1. An x-ray window comprising:  
a film spanning an aperture of a frame;  
the film across the aperture has  $\geq 70$  mass percent carbon;  
 $3 \mu\text{m} \leq T_{11} \leq 100 \mu\text{m}$ , where  $T_{11}$  is a maximum thickness of the film across the aperture;  
the film includes a polymer layer on a graphite layer; and  
 $T_{21}/T_{22} > 1$ , where  $T_{21}$  is a thickness of the graphite layer and  $T_{22}$  is a thickness of the polymer layer.
2. The x-ray window of claim 1, wherein the polymer layer faces a vacuum and the graphite layer faces ambient pressure.
3. The x-ray window of claim 1, wherein the polymer layer adjoins the graphite layer.
4. An x-ray device comprising:  
an x-ray window mounted to a frame;  
the x-ray window including a film spanning an aperture of a frame;  
the film across the aperture has  $\geq 70$  mass percent carbon; and  
 $3 \mu\text{m} \leq T_{11} \leq 100 \mu\text{m}$ , where  $T_{11}$  is a maximum thickness of the film across the aperture.
5. The x-ray device of claim 4, wherein the aperture is void of solid material except for the film.

## 6

6. The x-ray device of claim 4, wherein:  
the film includes a polymer layer on a graphite layer; and  
 $T_{21}/T_{22} > 1$ , where  $T_{21}$  is a thickness of the graphite layer and  $T_{22}$  is a thickness of the polymer layer.

7. The x-ray device of claim 6, wherein:

$2 \mu\text{m} \leq T_{21} \leq 25 \mu\text{m}$ ; and  
 $20 \text{ nm} \leq T_{22} \leq 500 \text{ nm}$ .

8. An x-ray window comprising:

a film including a polymer layer on a graphite layer; and  
 $T_{21}/T_{22} > 1$ , where  $T_{21}$  is a thickness of the graphite layer and  $T_{22}$  is a thickness of the polymer layer.

9. The x-ray window of claim 8, wherein the film has  $\geq 70$  mass percent carbon.

10. The x-ray window of claim 8, wherein  $3 \mu\text{m} \leq T_{11} \leq 100 \mu\text{m}$ , where  $T_{11}$  is a maximum thickness of the film.

11. The x-ray window of claim 8, wherein the polymer layer includes polyimide.

12. The x-ray window of claim 8, wherein the polymer layer faces a vacuum and the graphite layer faces ambient pressure.

13. The x-ray window of claim 8, wherein the polymer layer adjoins the graphite layer.

14. The x-ray window of claim 8, wherein the film has  $\geq 80$  mass percent carbon.

15. The x-ray window of claim 8, wherein  $T_{21}/T_{22} \geq 10$ .

16. The x-ray window of claim 8, wherein  $T_{21}/T_{22} \geq 50$ .

17. The x-ray window of claim 8, wherein  $T_{21}/T_{22} \leq 500$ .

18. The x-ray window of claim 8, wherein:

$2 \mu\text{m} \leq T_{21} \leq 25 \mu\text{m}$ ; and  
 $20 \text{ nm} \leq T_{22} \leq 500 \text{ nm}$ .

19. The x-ray window of claim 8, wherein the film consists essentially of graphite and polyimide.

20. The x-ray window of claim 8, wherein the film is planar across its width.

\* \* \* \* \*